

## 1

3,079,255

## PROCESSES OF DEVELOPING EXPOSED SILVER HALIDE PHOTOGRAPHIC EMULSIONS AND COMPOSITIONS FOR USE THEREIN

Ottmar Wahl, Baden-Baden, and Karl-Heinz Menzel, Kolin-Mülheim, Germany, assignors to Agfa Aktiengesellschaft, Leverkusen, Germany, a corporation of Germany

No Drawing. Filed Nov. 6, 1959, Ser. No. 851,267  
Claims priority, application Germany Nov. 12, 1958

11 Claims. (Cl. 96—55)

This invention relates to novel heterocyclic silver halide developer substances.

It has long been known that aromatic diamines, amino-phenols and aromatic o- and p-dihydroxy compounds are capable of developing photographic silver halide emulsions containing a latent image. Recently, photographic developer substances derived from heterocyclic basic substances, such as pyrazolones, pyrazolines and pyrazolidones, have acquired practical importance.

It has now been found that pyrazolino-benzimidazole compounds in which the methylene group of the pyrazolino nucleus is substituted by an amino group are valuable new silver halide developer substances. By way of example these new developer substances correspond to the general formula:



wherein R represents a hydrogen atom, or the carboxy, or amino-carbonyl ( $\text{NH}_2\text{CO}-$ ) radicals or a monovalent organic radical, such as an alkyl having 1 to 12 carbon atoms (methyl, ethyl, propyl, butyl); aryl (phenyl, aminophenyl, acyl-aminophenyl); aralkyl (benzyl); cycloalkyl (cyclohexyl); a heterocyclic radical ( $\alpha$ -furyl,  $\gamma$ -pyridyl),  $\alpha\text{-COOR}'$ ,  $-\text{NR}'\text{R}''$  or  $-\text{OR}''$  group in which R' and R'' each represent a hydrogen atom or an alkyl radical and the benzene ring (designated A in the foregoing formula) may be substituted by an alkyl, aryl or aralkyl radical as defined above, a halogen atom, an alkoxy, aroxy, OH, NH<sub>2</sub>, COOH or SO<sub>3</sub>H group or may be condensed with a further benzene ring which in its turn may be substituted.

These new heterocyclic developer substances are characterized inter alia by the fact that their very good developing properties are also maintained if carboxyl or sulphonic acid groups are introduced into the molecule, whereas with most developer substances containing amido groups, the developing activity is very greatly reduced by the introduction of acid groups.

An additional advantage of the new developer substances is that they are unobjectionable physiologically.

The amino-pyrazolino-benzimidazoles may be prepared by introducing an amino group into the pyrazolino-benzimidazoles described in our copending United States patent application Serial No. 819,066, filed June 9, 1959, by treating them in an acid aqueous solution with nitrous acid followed by reduction at temperatures of about 0 to 10° C., as for instance by means of hydrogen in the presence of a catalyst, such as Raney nickel. Alternatively the aforementioned pyrazolino-benzimidazoles may be coupled in an alkaline to neutral aqueous solution with diazonium salts and the resulting products reduced as disclosed to give the amido pyrazolino-benzimidazoles.

The aqueous solutions of the new heterocyclic compounds develop exposed silver halide emulsion layers into

## 2

strong silver images in the presence of alkali, such as alkali-metal carbonates or hydroxides, the pH values of the solutions being preferably adjusted to about 10-12. The solutions may contain the usual preservatives or anti-oxidants, such as sodium sulfite, sodium bisulfite, sodium metabisulfite or the corresponding potassium salts, preferably in amounts of 1 to 10 grams per liter of solution.

It has further been found that the new developer substances are excellently suitable for use as color developers in the process of chromogenic development. In this process the oxidation products which are formed during the development of the latent silver image react with the color couplers which are present to form dyestuffs. As color couplers, it is possible to use any of the known color couplers described in the literature which can react with the oxidation product of a primary aromatic amino developer to yield a dyestuff, such as aromatic amines, and phenols, naphthols, pyrazolones, oxazolones, cyanoacetic acid and acetoacetic acid or aryl acetic acid esters and amides, 1,3-diketones and hydroxythionaphthalenes. Typical color couplers or coupling compounds are exemplified by the formulae hereinafter, designated I to XI. Depending on the choice of the color couplers, it is possible to produce a wide range of colors, hues, and chromas from yellow through red and blue to green.

The particular advantage of the image dyestuffs obtained in color development using the new aminopyrazolino-benzimidazoles lies in the fact that they form metal dyestuff complexes with numerous metals in the form of their salts or soluble complex compounds, which complexes are characterized by high fastness to light. The complex may be produced either by treating the finally developed color images with a metal salt or soluble metal complex compound or by adding suitable soluble metal compounds during the color development. The metal complex formation is in many cases associated with a change in the color. Suitable metal salts are, for instance, the sulphates, chlorides and nitrates of Cr, Cu, Ni, Zn, Mn, Mg, Cd, Ca, Sr, Ba, which salts are preferably used in the form of 5% aqueous solutions, as illustrated in Example 5 hereinafter.

In the accompanying table are listed for a large number of color components the colors or hues that are formed during the color development with the new developers, and also the colors or hues which may be obtained by treatment with individual metal salts. In this table are also included the colors or hues produced when these color couplers are subjected to subsequent treatment with alkalis.

## EXAMPLE 1

An exposed photographic silver chlorobromide emulsion on a paper support is developed in a developing solution having the following composition:

55 5 g. of developer A or 7.5 g. of developer B (the preparation of developer A (4-aminopyrazolino[1.5:1'.2']-benzimidazole-3-carboxylic acid) and developer B (3-phenyl-4-aminopyrazolino[1.5:1'.2']benzimidazole-5-sulphonic acid) are described following Example 8 hereinafter)

75 g. of potassium carbonate

2 g. of sodium sulphite

2.5 g. of potassium bromide

1.2 g. of hydroxylamine sulphate  $[(\text{NH}_2\text{OH})_2\cdot\text{H}_2\text{SO}_4]$

2 g. of potassium hexametaphosphate

1000 cc. of water

The material is thereafter rinsed and fixed in the usual manner. A strong silver image is obtained.

## EXAMPLE 2

A photographic silver iodobromide emulsion layer on

## 3

a film support is exposed and developed in a developer having the following composition:

|                                                                                                                                                                                   |    |
|-----------------------------------------------------------------------------------------------------------------------------------------------------------------------------------|----|
| 1 g. of p-methylaminophenol sulphate                                                                                                                                              |    |
| 13 g. of sodium sulphite                                                                                                                                                          |    |
| 3 g. of developer B (3-phenyl-4-aminopyrazolino-[1.5:1'.2']benzimidazole-5-sulphonic acid, the preparation of which is described following Example 8 and developer A hereinafter) |    |
| 26 g. of sodium carbonate                                                                                                                                                         |    |
| 1 g. of potassium bromide                                                                                                                                                         | 10 |
| 1000 cc. of water                                                                                                                                                                 |    |

After the usual rinsing and fixing, a strong silver image is obtained.

## EXAMPLE 3

A photographic silver bromide emulsion layer which contains one of the diffusion-resisting color couplers I-VII (represented by formulae following Example 12 hereinafter) is exposed and developed in the developing solution described in Example 1. It is then rinsed, bleached and fixed in the usual manner. Details concerning the colors of the images thus obtained are included in the table hereinafter.

## EXAMPLE 4

The processing is initially as described in Example 3. Thereafter, the material is washed for 5 minutes in a 10% sodium hydroxide solution and thereafter rinsed for 2 minutes. The hues of the resulting color images are indicated in the table hereinafter.

## EXAMPLE 5

A photographic silver bromide emulsion layer which contains one of the color couplers I-VII (represented by formulae following Example 12 hereinafter) is initially processed as described in Example 3. The material is then washed for 5 minutes in a 5% magnesium sulphate solution or 5% zinc sulphate solution or 5% cobalt sulphate solution or a 5% nickel sulphate solution and thereafter rinsed for 5 minutes. Depending on which bath is used, color images having the colors indicated in the table hereinafter are obtained with the different color couplers.

## EXAMPLE 6

A photographic silver bromide emulsion layer which contains one of the color couplers I-VII (represented by formulae following Example 12 hereinafter) is initially processed as described in Example 3 and thereafter washed for 5 minutes in an ammoniacal 1% copper sulphate solution. It is then rinsed for 5 minutes and color images are obtained, the color of which is specified in the table hereinafter.

## EXAMPLE 7

The photographic material of Example 5 is initially processed as described in Example 5. It is thereafter washed for 5 minutes in a 10% sodium hydroxide solution and then rinsed for 2 minutes. There are obtained color images, the colors of which, when using magnesium sulphate solution, are set out in the table hereinafter.

## EXAMPLE 8

A photographic silver iodobromide emulsion layer coated on a film support is exposed and developed at 20° C. in a developer having the following composition:

|                                                                                                                                                                                    |  |
|------------------------------------------------------------------------------------------------------------------------------------------------------------------------------------|--|
| 38 g. of sodium sulphite (anhydrous)                                                                                                                                               |  |
| 25 g. of potassium carbonate                                                                                                                                                       |  |
| 37 g. of developer B (3-phenyl-4-aminopyrazolino-[1.5:1'.2']benzimidazole-5-sulphonic acid, the preparation of which is described following Example 8 and developer A hereinafter) |  |
| 0.275 g. of 1-phenyl-3-pyrazolidone                                                                                                                                                |  |
| 2.5 g. of sodium hydroxide                                                                                                                                                         |  |
| 4 g. of potassium bromide                                                                                                                                                          |  |
| 0.275 g. of 1,2,3-benzotriazole                                                                                                                                                    |  |
| 1000 cc. of water                                                                                                                                                                  |  |

## 4

The material is thereafter rinsed and fixed in the usual manner. The silver image thus obtained is twice as fast as a silver image obtained under comparable conditions in a developer in which the developer B had been replaced by an equimolar amount of hydroquinone.

The developer substances mentioned in the foregoing examples (1, 2, and 8) can be prepared as follows:

*Developer A: 4-amino-pyrazolino[1.5:1'.2']-benzimidazole-3-carboxylic acid.* —10 g. of pyrazolinobenzimidazole-3-carboxylic acid are dissolved in 50 cc. of a 10% aqueous sodium hydroxide solution and 3.8 g. of sodium nitrite are added thereto. The solution thus obtained is introduced dropwise at a temperature of from 0° C. to 5° C. into 30 cc. of 20% hydrochloric acid. The nitroso product is filtered with suction, dissolved in isopropanol with addition of ammonia (pH 8) and hydrogenated in the presence of Raney nickel at 50° C. and 50 atm. gauge. The product is filtered into 40% acetic acid and filtered off with suction.

Yield: 7 g.

The pyrazolinobenzimidazole-3-carboxylic acid is obtained as follows:

24 g. of 1-(o-aminophenyl)-carboxy-pyrazolone-5 obtained according to German Patent No. 1,046,496 are heated at 140° C. with 9.5 cc. of aniline and 18.5 g. of aniline hydrochloride for 2 hours. The melt is treated with 50 cc. of methanol, and sucked off after cooling.

Yield: 12 g. When heated, decomposition of the compound begins at 270° C.

*Developer B: 3-phenyl-4-amino-pyrazolino[1.5:1'.2']-benzimidazole-5'-sulphonic acid.* —12 g. of 3-phenyl-pyrazolinobenzimidazole-5'-sulphonic acid are dissolved in 50 cc. of 10% sodium hydroxide solution and 27 cc. of a 10% sodium nitrite solution are added thereto. The solution is added dropwise at a temperature of from 0° C. to 5° C. to 50 cc. of a 20% solution of sulphuric acid. The nitroso product is separated by suction filtration and dissolved in 150 cc. of isopropanol and 50 cc. of a 25% solution of ammonia (pH 8). Hydrogenation is carried out at 50° C. and 50 atm. gauge in the presence of Raney nickel, and the substance is recovered by acidification of the solution with 150 cc. of 20% sulphuric acid and suction filtration.

Yield: 8 g.

The 3-phenyl-pyrazolinobenzimidazole-5'-sulphonic acid is obtained as follows:

33 g. of 1-(o-amino-p-sulphophenyl)-3-phenylpyrazolone-5 obtained according to German Patent No. 1,046,496 are heated at 160° C. with 12 g. of m-toluidine for 2 to 3 hours. The melt is stirred with diluted hydrochloric acid and sucked off.

Yield: 30 g. When heated, decomposition of the compound begins at 310° C.

## EXAMPLE 9

*3-Carboxy-4-Amino-Pyrazolino-[1.5:1'.2']-Benzimidazole-5'-Sulphonic Acid*

9 g. of 1-(2'-amino-4'-sulphonic acid)-phenylpyrazolone-5-carboxylic acid-3 are heated at 170° C. with 10 cc. of aniline for 2 hours. After cooling to room temperature, the melt is stirred with 20% hydrochloric acid, whereby about 5 g. of 3-carboxy-pyrazolinobenzimidazole-5'-sulphonic acid separate. This compound is recovered by suction filtration.

Decomposition of the compound begins at 320° C.

5.9 g. of the latter compound are dissolved in 8 cc. of a 10% aqueous sodium hydroxide solution, mixed with a 10% solution of sodium nitrite, added at a temperature 10° C. to 0° C., followed by treatment with 30 cc. of methanol, after which the solution is rendered alkaline with aqueous ammonia. The nitroso product formed is mixed with 20 cc. of water and hydrogenated in the presence of Raney nickel at a temperature of 50° C. and a pressure of 50 atm. The resulting solution is acidified with 5 cc. of 20% sulphuric acid, whereby about 4 g. of

3-carboxy-4-amino-pyrazolinobenzimidazole-5'-sulphonic acid crystallize.

When heated decomposition of the compound begins at 280° C.

EXAMPLE 10

4-Amino-Pyrazolino-[1.5:1'.2']-Benzimidazole-3,5'-Dicarboxylic Acid

10.4 g. of 1-(2'-amino-4'-carboxy)-phenyl-pyrazolone-5-carboxylic acid-3 are heated at 170° C. with 5 g. of aniline hydrochloride and 8 cc. of aniline for 2 hours. When treating with 100 cc. of methanol about 8 g. of pyrazolinobenzimidazole-3,5'-dicarboxylic acid separate which are isolated by filtration.

When heated, decomposition of the compound begins at 270° C.

12 g. of the latter compound are dissolved in 100 cc. of a 4% aqueous sodium hydroxide solution, mixed with 35 cc. of a 10% aqueous sodium nitrite solution and added dropwise to 50 cc. of a 20% solution of sulphuric acid at a temperature of -5° C. to 0° C. The nitroso product obtained is separated by suction filtration and dissolved in a mixture of 100 cc. of water, 100 cc. of methanol and 15 cc. of ammonia (25%). In the presence of Raney nickel the product is hydrogenated at 50° C. and 50 atm. Thereafter, the product is acidified with 100 cc. of 20% sulphuric acid, separated by suction filtration and washed with isopropanol. About 9 g. of 4-amino-pyrazolinobenzimidazole-3,5'-dicarboxylic acid are obtained.

EXAMPLE 11

3-Methyl-4-Aminopyrazolino-[1.5:1'.2']-Benzimidazole

34 g. of 3-methylpyrazolinobenzimidazole are dissolved in 75 cc. of 20% sulphuric acid. At a temperature of -5° C. to 0° C., 140 cc. of a 10% aqueous sodium nitrite solution are added dropwise. The nitroso-product is separated by suction filtration washed with water, ground with 250 cc. of methanol in the cold, and separated by suction filtration once again. The nitroso product is hydrogenated after being mixed with 350 cc. of methanol and 50 cc. of 25% ammonia in the pressure of Raney nickel at a temperature of 50° C. and a pressure of 50 atm., acidified with 250 cc. of 20% sulphuric acid, cooled and separated by suction filtration. In order to purify the amino product thus obtained, it is recrystallized from 2000 cc. of water in the presence of activated carbon.

Yield: 20 g. When heated, decomposition of the compound begins at 175° C.

The 3-methylpyrazolinobenzimidazole is obtained from 1-o-aminophenyl-3-methylpyrazolone by melting with aniline according to the procedure described hereinbefore in Example 9.

EXAMPLE 12

4-Aminopyrazolino-[1.5:1'.2']-Benzimidazole-3-Carboxamide

50 g. of pyrazolinobenzimidazole-3-carboxylic acid are boiled in 500 cc. of a 3% solution of hydrochloric acid in methanol for 8 hours. On cooling, 40 g. of pyrazolinobenzimidazole-3-carboxylic acid methyl ester crystallize out (melting point: 262° C.). 34 g. of the methyl ester thus obtained are heated at 80 to 85° C. with 250 cc. of 25% aqueous ammonia for 8 hours in an autoclave. The reaction product is recovered by suction filtration and extracted with methanol. There are obtained about 21 g. of pyrazolinobenzimidazole-3-carboxamide (melting point: 271° C.).

20 g. of the amide thus prepared is mixed with 50 cc. of 20% sulphuric acid and treated with 75 cc. of a 10% aqueous sodium nitrite solution at 0 to 5° C. The green nitroso product obtained is filtered off, washed with water, and hydrogenated in 250 cc. of methanol and 70 cc. of 25% ammonia in the presence of Raney nickel at 50° C. and 50 atm. After filtering the reaction mixture the filtrate is acidified with 20% sulphuric acid, whereby the

4-aminopyrazolinobenzimidazole-3-carboxamide precipitates as the sulphate. In order to purify the product, it is extracted with 500 cc. of methanol.

Yield: 22 g. (melting point: 220° C.).

The compounds of Examples 9 to 12 are silver halide black/white and color developers, and may be used instead of the developers A and B in the solutions of Examples 1, 2 and 8.

The compounds whose formulae follow are diffusion-resistant color couplers or coupling compounds that were referred to in the description hereinbefore. The compounds designated from I to VII were referred to specifically in Examples 3 to 7. These compounds are referred to in the table which follows hereinafter by these Roman-numeral designations.





ma-pyridyl, the benzene ring A being a benzene ring selected from the group consisting of an unsubstituted benzene ring, and a benzene ring substituted by at least one radical selected from the group consisting of carboxy and sulfo.

4. A process as defined in claim 1 in which the silver halide developer substance is 4-amino-pyrazolino-[1.5:1'2']-benzimidazole-3-carboxylic acid.

5. A process as defined in claim 1 in which the silver halide developer substance is 3-phenyl-4-aminopyrazolino-[1.5:1'.2']-benzimidazole-5'-sulphonic acid.

6. A process as defined in claim 1 in which the silver halide developer substance is 3-carboxy-4-amino-pyrazolino[1.5:1'.2']-benzimidazole-5'-sulphonic acid.

| Developer | p-Diethyl-aminoaniline | A       | A, 10% Na <sub>2</sub> CO <sub>3</sub> | A, Mg salts     | A, Mg salts, 10% Na <sub>2</sub> CO <sub>3</sub> | A Zn salts    | A, Co salts   |
|-----------|------------------------|---------|----------------------------------------|-----------------|--------------------------------------------------|---------------|---------------|
| I         | Cyan                   | Blue    | Cyan                                   | Blue            | Cyan                                             | Blue          | Blue          |
| II        | do                     | do      | do                                     | do              | do                                               | Cyan          | Blue-grey     |
| III       | Magenta                | Orange  | Blue                                   | Orange          | Violet                                           | Reddish brown | Violet        |
| IV        | do                     | Red     | Red                                    | Magenta         | Magenta                                          | Magenta       | Magenta       |
| V         | Red                    | Yellow  | Magenta                                | Brownish yellow | do                                               | Brown         | Reddish brown |
| VI        | Yellow                 | do      | Yellow                                 | Yellow          | Yellow                                           | Yellow        | Yellow        |
| VII       | do                     | Brown   | Violet                                 | Brown           | Violet                                           | Brown         | Violet        |
| VIII      | Cyan                   | Magenta | Magenta                                |                 |                                                  |               |               |
| IX        | Magenta                | Blue    |                                        |                 |                                                  |               |               |
| X         |                        | Green   |                                        |                 |                                                  |               |               |
| XI        | Cyan                   | Blue    |                                        |                 |                                                  |               |               |

We claim:

1. A process for developing an exposed photographic silver halide emulsion which comprises developing the said exposed photographic silver halide emulsion in an aqueous alkaline solution of a silver halide developing substance that comprises a 4-aminopyrazolino[1.5:1'2']-benzimidazole.

2. An aqueous alkaline color developer consisting essentially of a solution of a 4-amino-pyrazolino-[1.5:1'.2']-benzimidazole and a color-coupler capable of reacting with the oxidation product of a primary aromatic amine developer to form a dyesuff.

3. A process for developing an exposed silver halide emulsion as defined in claim 1 in which the silver halide developer substance corresponds to the tautomeric formulae:



40 7. A process as defined in claim 1 in which the silver halide developer substance is 4-amino-pyrazolino-[1.5:1.2']-benzimidazole-3,5'-dicarboxylic acid.

8. A process as defined in claim 1 in which the silver halide developer substance is 3-methyl-4-aminopyrazolino-[1.5:1'.2']-benzimidazole.

45 9. A process as defined in claim 1 in which the silver halide developer substance is 4-aminopyrazolino-[1.5:1'.2']-benzimidazole-3-carboxamide.

10. A process as defined in claim 1 in which the silver halide emulsion layer is contacted with the developer substance and with a color coupler which is capable of reacting with the oxidation product of a primary aromatic amine developer to form a dyestuff, thereby producing a combined silver and dyestuff image.

55 11. A process as defined in claim 1 in which the alkaline solution has a pH value between about 10 and about 12.

**References Cited in the file of this patent**

UNITED STATES PATENTS

|           |                  |                |
|-----------|------------------|----------------|
| 2,588,538 | Kendall          | Mar. 11, 1952  |
| 2,726,248 | Kendall et al.   | Dec. 6, 1955   |
| 2,817,654 | Grandjean et al. | Dec. 24, 1957  |
| 2,840,567 | Marsch et al.    | June 24, 1958  |
| 2,852,375 | Tinker           | Sept. 16, 1958 |

UNITED STATES PATENT OFFICE  
CERTIFICATE OF CORRECTION

Patent No. 3,079,255

February 26, 1963

Ottmar Wahl et al.

It is hereby certified that error appears in the above numbered patent requiring correction and that the said Letters Patent should read as corrected below.

Column 2, line 58, and column 3, lines 6 and 68, for "benzimidazole-5-", each occurrence, read -- benzimidazole-5'; column 3, lines 28 and 56, for "hydroxide", each occurrence, read -- carbonate --; column 4, line 23, before "carboxy" insert -- 3- --; line 68, after "temperature" insert -- of --; same column 4, line 69, before ", followed" insert -- to aqueous acid --; columns 7 and 8, in the headings to the first columns of each of the two tables, for "Developer", each occurrence, read -- Color coupler --.

Signed and sealed this 14th day of April 1964.

(SEAL)

Attest:

ERNEST W. SWIDER

Attesting Officer

EDWARD J. BRENNER

Commissioner of Patents